

April 2, 1968

R. C. SABINS

3,376,209

ANODE FORMED OF LEAD BASE AND DURIIRON

Filed Nov. 6, 1964



Fig. 2



Fig. 4



Fig. 1



Fig. 3

INVENTOR  
ROLLAND C. SABINS

Warren T. Schmiding  
ATTORNEY

# United States Patent Office

3,376,209

Patented Apr. 2, 1968

1

3,376,209

## ANODE FORMED OF LEAD BASE AND DURIRON

Roland C. Sabins, 522 Catalina Blvd.,  
San Diego, Calif. 92106

Continuation-in-part of application Ser. No. 407,302,  
Oct. 29, 1964. This application Nov. 6, 1964, Ser.  
No. 412,873

10 Claims. (Cl. 204—196)

The present invention relates to an electrolytic system and to an anode for said system. More particularly, the present invention is directed to an electrolytic system for preventing galvanic dissolution of cathodic material and is directed also to an anode which is relatively inexpensive yet has the characteristics of expensive substances such as platinum.

The present invention is a continuation-in-part of my copending application Ser. No. 407,302, filed Oct. 29, 1964, now abandoned.

In practicing the present invention, an extraneous source of direct current is impressed upon the system to increase the potential of the cathode to above its dissolution potential.

It is known that when an attempt is made to use a single body of some substances, such as lead, as an anode in a galvanic system employing, for example, sea water as the electrolyte, such substances become passive to the flow of current and therefore can function as an anode only during the period prior to the substances becoming passive.

I have discovered that by physically associating several of the elements, such as iron and silicon in intimate contact with and exposed to the outer surface of such substance, such as lead, such mass becomes a composite anode and remains sufficiently active so that the entire outer surface thereof, which is exposed to the electrolyte, functions anodically and that such substance ceases to dissolve after being coated by a compound including the substances, such as lead, and the substances such as iron and silicon which are decomposed by an electric current while in the electrolyte.

Further features and the advantages of the present invention will be apparent from the following description, reference being had to the accompanying drawing wherein a preferred embodiment of the invention is illustrated.

In the drawing:

FIG. 1 is a diagrammatic view illustrating a galvanic system wherein my invention is employed;

FIG. 2 is a fragmentary view of a metallic structure of cathode material, as for example, the hull of a steel ship, together with the fragmentary view of the improved anode;

FIG. 3 is a sectional view of the anode taken on line 3—3 of FIG. 2; and

FIG. 4 is a fragmentary sectional view taken along line 4—4 of FIG. 2, but on a larger scale.

Referring more in detail to the drawing and particularly to FIGS. 2 and 3, I have shown a cathode at 20, which may be any metallic object or objects which is or are to be adapted to be polarized and in which it is desirable to maintain a substantially uniform polarization of the entire surface which could be affected by galvanic action. Thus, for example, the cathode may be the hull of a ship and is herein shown as such. The composite anode is shown at 22 and will be described more in detail hereinafter.

The electrolyte may be any suitable compound, such as water or earth. For illustrative purposes, the cathode is shown as embedded in an electrolyte, for example sea water, the level of which is indicated by the dot and dash lines 22.

2

The cathode 20, anode 22 and electrolyte are connected in galvanic relationship through a circuit including a source of direct current. This source of direct current is illustrated by two wires 24 and 26, 24 being connected to the negative terminal and 26 to the positive terminal of the source of direct current. The circuit includes a wire 24, ammeter 28, wire 30, variable resistance 32, wire 34, cathode 20, the electrolyte, anode 22 and wire 26.

To protect metal from corrosion, the relative potential at the surface of the metal must be increased to transpose the normal positive ionic surface state to an impressed negative ionic state. For example, a steel structure cathode has a potential of 630 millivolts with reference to a silver-silver chloride reference anode. It is known that to protect the ship's hull, made of steel, from corrosion in sea water, a potential should exist of approximately 890 millivolts, depending upon varying factors, and accordingly the potential of the steel cathode must be raised approximately 260 millivolts to prevent galvanic corrosion of dissolution of the metal, which corrosion or dissolution results in pitting. This increasing in potential is accomplished by subjecting the cathode to the electron flow in the external circuit. The variable resistance 32 is used to regulate the potential to that necessary for raising of the potential of the cathode.

The reference electrode is shown at 36 which is connected with the cathode 20 by wire 38, millivoltmeter 40 and wire 42.

Some compounds, and a number of the elements, enter a passive state when they are functioning as an impressed current anode in certain electrolytes subject to required current density and time. That is, the surface coating material becomes more passive to the passage of electrons when the electrolyte is decomposed by the current flowing therethrough, as for example, in the ionic exchange phenomena. In certain of these elements or compounds, the passivity thereof increases to such an extent that it substantially completely isolates the surface conductive of the electrode from the electrolyte environment. Such is true with respect to the metals aluminum, lead, and other metallic compounds.

I have discovered that by physically associating, with an anode 22 formed of a lead base, a small piece or small pieces of the elements iron and silicon at the surface of the lead, passivity of the anode 22 is checked, i.e., after a certain stage of decomposition of the electrolyte, no further dissolution of the lead takes place. Upon reaction with the electrolyte, a compound is formed in a thin layer only about the entire surface of the composite anode which is being subjected to the electrolyte. It is believed that this compound is a peroxide of lead. Due to the presence of the iron and silicon at the surface of the lead, the forming of the compound stops at a stage in which the entire surface of the whole anode functions as an anode but without further dissolution of the lead.

Thus, in effect, the entire surface of the relatively inexpensive lead functions to perform substantially the same service as an equal area of the highly expensive platinum in that it is relatively inert, yet functions as an anode.

My observation has been that the entire surface of the anode functions as an anode, since gases are evolved throughout this entire area, most of which gases as yet have not been identified but is chlorine as would be the case if the entire surface of the anode was platinum anode surface.

The iron and the silicon should be in intimate contact with the lead, that is, both of these elements should be fastened in some manner to the lead. The iron and silicon could be in the form of a unit and this composition can be pressed or clamped on to the lead. In one form of the

invention, balls, shots, or fine pieces of the composition 43 of iron and silicon are entered into the mold at the time that the lead is cast in the desired shape. The composition being less dense than lead, it will float to the top of the lead casting and therefore be exposed to the surface of the lead. These balls, shots, or pieces are in the form of a random pattern and the composition comprises 80% to 85% of iron and 15% to 10%, respectively, of silicon. The composite anode 22 need include less than one percent of the composition of iron and silicon for satisfactory results. Excellent results were achieved using lead and a composition sold under the trademark Durion.

Preferably the anode comprises a series of lead tubing or cables, having cast therein and at the surface thereof, the balls, shots, or pieces of the composition of iron and silicon. These lead cables are shown at 44. These cables 44, extend longitudinally and are suitably fastened to the cathode, herein shown as the outer side of the hull of the ship. They have a diameter of three-fourths inch, in actual practice. Vertically extending steel plates 48 in 10 are suitably welded to the outer surface of the hull. They are tapped and threaded as at 50 for receiving bolts 52. The composite anode 22 also includes a plurality of vertically extending anode parallel bars 54, each having a plurality of transverse or horizontally extending semi-circular grooves 56 for receiving the cables 44. These bars 54 are formed of the same material as the cables 44 and also carry at the surface thereof, the composition 15 iron and silicon. The anode including the cables 44 and the bars 54 are insulated from direct contact with the hull of the ship and likewise, the plates 48 by dielectric material such as vertically extending strips 58 and 60. The nylon strip 58 is provided with three transverse or 20 horizontally extending semi-circular grooves 46. The grooves 46 in the nylon strip 58 and grooves 56 in the bars 54 complement the cables 44. The nylon strip 60 is provided with semi-circular grooves 62 which extend transversely, i.e., horizontally and these grooves complement the periphery of the arcing shape of the bars 54. The bolts 52 pass through holes 64 and 66, respectively, in the nylon strips 58 and 60 and when fastened securely, 25 the composite anode including cables 44 and bars 54 are secured to the plate 48.

Steel bars 68 and 70 are disposed, respectively, above and below the anode and are welded to the outer surface of the hull and thereby assist in guarding the anode should the ship encounter wharfs or the like.

The coating is not shown in FIGS. 2 and 3, but is shown at 72 and the random dispersement of the composition of iron and silicon is shown at 43. While such dispersement is shown in elevation in FIGS. 2 and 3, such is for illustrative purpose only since the coating 72 covers the entire surface of the composite anode 22 as shown in FIG. 4.

The word "cable" as herein used may take various forms such as tubing, strands of wire, and may have shapes other than cylindrical.

Thus, it is apparent from the foregoing that I have materially reduced the cost of inert anodes since the same results are achieved for like amount of surfaces heretofore deemed necessary in noble metals such as platinum or lead alloyed with a noble metal,

While the method herein described constitutes a preferred method, it is to be understood that other methods may be adopted falling within the scope of the claims that follow.

I claim:

1. A control system for preventing corrosion of a metallic structure which is subjected to an electrolyte, comprising in combination:

(A) a source of direct current having the negative side thereof connected with the structure; and

(B) A composite anode connected to the positive side of said source of current and subjected to the electrolyte, said anode comprising a lead base and an alloy of iron and silicon in intimate contact with and exposed to the electrolyte at the outer surface of said lead base to maintain the anodic activeness of the entire surface of the lead base.

2. A system as defined in claim 1, in which said alloy comprises 80% to 85% iron and 15% to 10% of silicon.

3. A system as defined in claim 1, in which said alloy constitutes a fraction of one percent of the composite anode.

4. A system as defined in claim 1, in which said alloy constitutes a fraction of one percent of the composite anode, and in which said alloy comprises 80% to 85% iron and 15% to 10% of silicon.

5. A system as defined in claim 1, characterized in that the lead base is an elongated bar insulatingly fastened to the structure.

6. A system as defined in claim 1, characterized in that the structure is a hull of the ship and said anode is fastened to the hull substantially horizontally and below the water line.

7. A composite anode comprising:

(A) lead base;

(B) and an iron-silicon alloy exposed at the outer surface of the lead base.

8. An anode as defined in claim 7, in which the alloy constitutes a fraction of one percent of the composite anode.

9. An anode as defined in claim 8, in which the alloy comprises 80% to 85% iron and 15% to 10% silicon.

10. An anode as defined in claim 7, in which the alloy comprises 80% to 85% iron and 15% to 10% silicon.

#### References Cited

##### UNITED STATES PATENTS

|           |         |              |         |
|-----------|---------|--------------|---------|
| 546,328   | 9/1895  | Hoepfner     | 204—290 |
| 628,676   | 7/1899  | Pollak       | 136—76  |
| 1,302,959 | 5/1919  | Page         | 204—290 |
| 1,788,485 | 1/1931  | Gunderson    | 204—196 |
| 1,984,899 | 12/1934 | Smith        | 204—196 |
| 3,043,765 | 7/1962  | Bryan et al. | 204—196 |
| 3,108,939 | 10/1963 | Sabins       | 204—196 |
| 3,284,333 | 11/1966 | Parsi et al. | 204—196 |
| 3,294,667 | 12/1966 | Giuffrida    | 204—196 |

##### FOREIGN PATENTS

|    |        |         |          |
|----|--------|---------|----------|
| 60 | 77,881 | 10/1894 | Germany. |
|----|--------|---------|----------|

HOWARD S. WILLIAMS, Primary Examiner.

T. TUNG, Assistant Examiner.

UNITED STATES PATENT OFFICE  
CERTIFICATE OF CORRECTION

Patent No. 3,376,209

April 2, 1968

Rolland C. Sabins

It is certified that error appears in the above identified patent and that said Letters Patent are hereby corrected as shown below:

Column 1, line 51, "cathode" should read -- cathodic --; line 59, "3." should read -- 3, --; line 60, cancel "to"; line 61, cancel "be". Column 4, line 12, "pead" should read -- lead --.

Signed and sealed this 5th day of August 1969.

(SEAL)

Attest:

Edward M. Fletcher, Jr.

Attesting Officer

WILLIAM E. SCHUYLER, JR.

Commissioner of Patents